

## UNITED STATES PATENT OFFICE.

DANIEL C. BRUCE, OF NASHVILLE, TENNESSEE.

## COMPOSITION OF MATTER.

No Drawing.

Application filed July 29, 1926. Serial No. 125,828.

The invention is a filler of a soft putty consistency, and is designed to be used in connection with the application of cane fibre wall board, such as, and including, the wall board known as Celotex, and this invention is particularly for the purpose of filling the joints and covering the nail heads of the said wall board in walls and ceilings of buildings. The invention is designed, by its application 10 in the joints, to make a one-piece wall or ceiling so that the joints will have the appearance of the wall board itself; and if necessary the walls can be left either unpainted or covered with any solution or coating in the way of 15 paint or decorative wall covering.

The formula for preparing this composition is as follows:

Prepare a soap jelly by adding three ounces of white hard soap such as castile soap to two 20 quarts of water and heating near the boiling temperature till the soap dissolves.

Also prepare a starch dextrin paste adding 100 g. of cold water to a mixture of 80 g. starch and 20 g. powdered white dextrin. 25 Stir to a paste. Then add a solution of 20 g. borax and 40 g. glycerine in 700 g. of boiling water to the cold water paste and while the boiling liquid is being added stir the mixture until the milky streaks disappear. Add 4 g. 30 oil of cloves, and stir thoroughly.

After the starch-dextrin paste is cold, remove the skin that is formed on top and mix 200 g. of the paste with 2 g. of the soap jelly, 35 15 g. of Spanish whiting, 7½ g. of gasoline, and 7½ g. kerosene. This mass should be worked by stirring and kneading till the gaso-

line is worked into the mixture and the mass has a lard-like consistency.

To make the filler, mix the lard-like paste 40 with fibres obtained by shredding, sawing, filing, or boring the Celotex wall board in the proportion of 60 g. paste to 9 g. of fibres and knead thoroughly.

The formula hereinbefore described is 45 given in grams of weight, and the component parts are according to the following diagram.

|                    |                                             |        |    |
|--------------------|---------------------------------------------|--------|----|
| I. Soap jelly      | Soap                                        | 3 oz.  | 50 |
|                    | { Water                                     | 2 qts. |    |
| II. Starch dextrin | { Starch                                    | 80 g.  | 55 |
| paste              | { Dextrin                                   | 20 g.  |    |
|                    | { Water                                     | 100 g. | 60 |
|                    | { Borax                                     | 20 g.  |    |
|                    | { Glycerine                                 | 40 g.  | 65 |
|                    | { Water                                     | 700 g. |    |
|                    | Boiling when                                |        |    |
|                    | added to (a)                                |        |    |
|                    | Add oil of cloves 4 g. and stir thoroughly. |        |    |
|                    | Pour (b) into (a) and when cold remove      |        |    |
|                    | skin.                                       |        |    |
| III. Paste         | Paste II                                    | 200 g. | 70 |
|                    | Soap jelly I                                | 2 g.   |    |
|                    | Whiting                                     | 15 g.  | 75 |
|                    | Gasoline                                    | 7½ g.  |    |
|                    | Kerosene                                    | 7½ g.  |    |
| IV. Putty          | Paste III                                   | 60 g.  | 80 |
|                    | { Fibres                                    | 9 g.   |    |

I claim:

1. A filling composition consisting of an admixture of a soap jelly, a starch dextrin paste including borax, glycerine and oil of cloves, and comminuted fibrous material in the proportions specified.

2. A filling composition consisting of an admixture of soap jelly, a starch dextrin paste including borax and glycerine, and comminuted fibrous material in the proportions specified.

DANIEL C. BRUCE.